

F. C. WRIGHT.  
CACTUS LEATHER.  
APPLICATION FILED JAN. 15, 1908.

902,359.

Patented Oct. 27, 1908.



Witnesses

James F. Crown  
James Brausfield

Inventor

Frederick C. Wright.  
By Alexander Towell  
Attorneys

# UNITED STATES PATENT OFFICE.

FREDERICK C. WRIGHT, OF TUCSON, ARIZONA TERRITORY.

## CACTUS LEATHER.

No. 902,359.

Specification of Letters Patent.

Patented Oct. 27, 1908.

Application filed January 15, 1908. Serial No. 410,976.

To all whom it may concern:

Be it known that I, FREDERICK C. WRIGHT, of Tucson, in the county of Pima and Territory of Arizona, have invented certain new and useful Improvements in Cactus Leather; and I hereby declare that the following is a full, clear, and exact description thereof, reference being had to the accompanying drawings, which form part of this specification.

This invention is a novel artificial leather produced from vegetable growths of the cacti family, and its object is to produce a leather-like substance by tanning or treating slabs, layers, planks, or sheets cut from the cactus, which sections when treated and dried will have a close resemblance to leather and can in many instances be used as a substitute therefor, particularly where it is not subjected to very rough or hard usage, the product being specially useful in the arts, for fancy articles of manufacture such as furniture, frames, veneering, and many other purposes too numerous for specific mention.

The product of the invention is distinctively different from other imitation or artificial leathers, as the sections are tanned as cut from the cacti, and do not have to be produced by agglutination or compounding as the commonly known artificial leathers are made.

The invention will be more clearly comprehended from the following description and summarized in the claims; and in the accompanying drawings I have illustrated some forms of cacti from which such imitation leather has been made by me, and some of the preferred steps in its manufacture.

In carrying out my invention I preferably use the *Echinocactus wislizenii*, and varieties thereof, which are commonly known as niggerhead cactus, and grow in short thick stubs to a height sometimes of five feet or more, and fourteen inches or more in diameter. Other scientific names for this cactus are *E. emoryi* and *E. cylindraceus*. I however can use other varieties of cacti, preferring the larger growths, such as the Saguaro cactus, which grows very thick and sometimes to a height of forty feet or more.

In the drawings—Figure 1 represents an ordinary "niggerhead" cactus. Fig. 2 a Saguaro cactus. Figs. 3, 4 and 5 illustrate modes of cutting the cacti into sections pre-

paratory to treating same for leather. Fig. 6 represents a part of a Saguaro cactus showing its peculiar growth.

In carrying out my invention I first cut 60 the cactus plants into suitable lengths, and then cut these lengths into sections either transverse, as indicated in Fig. 3, or longitudinal, as indicated in Fig. 4; or into sheets by circumferential cuts, as in Fig. 5; or I 65 may cut the cacti into sections or blocks of any desired form and treat them. The sections or sheets of cacti are then placed in a tanning bath, which may be composed of the following ingredients in about the stated 70 proportions. Two ounces tannic acid. Forty pounds of glycerin. Twenty gallons of water.

The time in which the section should be left in the tanning solution will vary with 75 the thickness of the sections, but for sections or sheets like ordinary hide leather or skins in thickness, I have found about twelve hours immersion sufficient. After this treatment the sheets are taken out of the bath and 80 the excess moisture removed. The sheets may be pressed if desired for this purpose; or may be dried by exposure to sun, or artificially. The resultant product can then be stained, coated with oil, or water-proofed 85 by the processes already known for treating leather and artificial leather.

If desired the sections may be pressed or rolled before immersion in the bath, to expel water therefrom; and the tanning solution may be varied. The essential feature of the invention being the production of imitation leather, or a product resembling leather in appearance, from cactus growths, 90 without disintegration of such growths.

The heart of the Saguaro cactus is peculiar, and as shown in Fig. 6 of drawings it is composed of an annular series of rods *e*, inclosing a center pith *f*, and surrounded by a pith or pulp *g* filling the space between the 95 core and the outer shell or rind *h* of the body. The leather formed from the part *g* will be of different texture from that formed by part *f*, and will be translucent when tanned, unless cut very thick. The part *e* can be removed and tanned in any desired lengths, and if the rods are not first separated they will be united when tanned by the intervening fibers, and form a very tough ridged or fluted material, which may be worked into 100 many fancy articles.

I do not wish to confine myself to the par-

- ticular tanning bath or solution above named, for it can be varied, and the essential product of the invention obtained; and the resultant product, which I term "cactus leather" may be worked into various articles for which leather is now used. For example, I have found that a solution of ten pounds of gum arabic and ten pounds of glycerin in twenty gallons of water, will produce a very good imitation leather from cactus fiber if the cactus sheets are immersed therein about twelve hours. The brittleness of the leather will be increased if the proportion of glycerin is reduced.
- 15 The use of tannic acid is not absolutely necessary for tanning the cactus fiber, but I prefer it in the first solution to impart a tan color to the product and give it a leather odor. Other substitutes may be employed 20 for obtaining the desired color and odor.
- Having described my invention what I claim as new and desire to secure by Letters Patent is:
1. As a new article of manufacture, the imitation leather product obtained by treating cactus, substantially as set forth.
2. As a new article of manufacture, an artificial or imitation leather, consisting of sections of cactus plants treated substantially as described. 30
3. The herein described process of treating cactus consisting in cutting the cactus into sections of desired shape and form, then treating such sections with a preserving and toughening solution, and finally drying the product, substantially as described. 35
4. The herein described process of producing imitation leather from cactus, consisting in cutting the cactus plant into sections of the desired size and thickness, immersing such sections in a tanning bath or solution until cured, removing the sections from the bath and expelling the surplus moisture or solution therefrom, substantially as described. 40
- In testimony that I claim the foregoing as my own, I affix my signature in presence of two witnesses.

FREDERICK C. WRIGHT.

Witnesses:

T. R. BLANBERG,  
MONTE MANSELD.